

1

3,552,966

## COLOR PHOTOGRAPHIC DEVELOPMENT PROCESS

Gerhard Kuhn, Leverkusen, Albin Graf, Munich, Franz Moll, Cologne-Stammheim, and Rigobert Otto, Leverkusen, Germany, assignors to Agfa-Gevaert Aktiengesellschaft, Leverkusen, Germany, a corporation of Germany

No Drawing. Filed May 24, 1967, Ser. No. 640,825  
Claims priority, application Germany, July 2, 1966,

A 52,918

Int. Cl. G03c 7/30, 7/40

U.S. CL. 96—54

3 Claims

### ABSTRACT OF THE DISCLOSURE

The sensitivity of color photographic material is increased and its image grain size reduced by treating the material after color development and before bleaching, with an aqueous alkaline bath containing per liter 0.01 to 1.0 gram of a black-white developer of the p-aminophenol or 1-phenylpyrazolidone series. The bath may contain antioxidants, alkali metal sulfites, sequestering agents and stabilizers.

The invention relates to an improved process for developing color photographic materials by using after color development a bath containing black-white developers.

Many different ways of modifying the color development of color-photographic materials are known for achieving improved color densities, sensitivity, etc. Thus, for example, it has been stated that when developers that are used for black-white films, such as aminophenols, are added to a conventional color-forming developer, a higher yield of dye is observed in the developing of color photographic layers, especially in the blue-green layer. However, this is generally accompanied by undesirably coarsening of the grain and in addition, the improvement in the cyan density is in many cases associated with reduction of the magenta density.

It is also known to enhance the sensitivity of the color-photographic material by additional baths which are to be applied after color development. These baths generally contain inorganic salts, for example, potassium bromide. This modified procedure, also however, leads to a coarser dye grain, which is a serious disadvantage from the point of view of the quality of the final dye image.

It is the object of the present invention to improve the processing of color photographic materials, so as to obtain an enhanced sensitivity with as small as possible grain size.

We now have found that the sensitivity of color photographic materials, in particular color negative films, is substantially enhanced if the exposed and developed material is treated with an after-treatment bath which contains black-white developers, especially of the aminophenol type or of the pyrazolidone type. At the same time, a dye image of considerably finer grain is obtained.

Suitable developers of the p-aminophenol series are the following:

p-aminophenol  
p-N-methylaminophenol  
p-N-2-hydroxyethylaminophenol  
1-hydroxy-3,4-diaminobenzol  
1-hydroxy-2,5-dimethyl-4-aminobenzol  
1-hydroxy-2-methyl-4-aminobenzol  
1-hydroxy-2-hydroxymethyl-4-aminobenzol  
1-hydroxy-3-methyl-4-aminobenzol.

Suitable developers of the 1-phenylpyrazolidone series are described in U.S. Pat. No. 2,289,367.

The after-treatment bath to be used according to the invention contains, apart from the black-white developer,

2

the usual further additives, the concentrations of which are not critical and depend on the kind of the color-photographic material processed. We have found that generally after-treatment baths of the following composition are quite adequate to accomplish the desired results:

|    |                                                                                                                                  | G.       |
|----|----------------------------------------------------------------------------------------------------------------------------------|----------|
| 5  | Black-and-white developer                                                                                                        | 0.01-1   |
|    | Preferably                                                                                                                       | 0.05-0.5 |
| 10 | Antioxidants such as hydroxylamine                                                                                               | 1-4      |
|    | Alkali metal sulfites                                                                                                            | 2-10     |
|    | Sequestering agents such as sodium hexameta phosphate                                                                            | 1-5      |
|    | Stabilizers such as potassium bromide                                                                                            | 0.2-0.5  |
| 15 | Alkalizing agents such as sodium or potassium carbonate, alkali metal phosphates or borates, alkali metal hydroxides or the like | 10-20    |
|    | Water up to 1 l.                                                                                                                 |          |

The after-treatment bath according to the invention 20 preferably has a pH of between 8 and 12 and in particular between 9 and 10.

The color developers to be used in the process according to the invention have the usual composition. As color 25 developers it is preferred to use developers of the p-phenylene diamine type. The color developer may also contain development accelerators such as quaternary ammonium salts, polyethyleneoxides or derivatives such as spirocyclic phosphoric esters of polyethyleneglycol. Black-white developer compounds may be added to the color developer.

### EXAMPLE

Samples of a multi-layered color photographic material of the usual composition with a red-sensitive silver halide gelatin emulsion layer arranged on the support, which layer contains color couplers that react with the oxidation product of the color-forming developer to form the cyan image, a green-sensitive silver halide gelatin emulsion layer arranged on the red-sensitive layer, which green-sensitive 35 layer contains color couplers for the magenta image, a yellow filter layer and uppermost a silver halide gelatin emulsion layer containing color couplers for producing the yellow image, are exposed behind step wedges in a conventional sensitometer and processed as follows:

|                                                      | Processing Method A | G.  |
|------------------------------------------------------|---------------------|-----|
| Color developer:                                     |                     |     |
| Sodium hexametaphosphate                             | -----               | 2   |
| p-N,N-diethylphenylenediamine                        | -----               | 2   |
| Hydroxylamine sulfate                                | -----               | 2   |
| 50 Sodium sulfite sicc.                              | -----               | 2   |
| KBr                                                  | -----               | 1.5 |
| Potassium carbonate                                  | -----               | 50  |
| Make up to 1000 ml., the pH being 10.8.              |                     |     |
| 55 Development time 10 minutes at 22° C.             |                     |     |
| Short stop bath—treatment time 4 minutes:            |                     |     |
| Sodium acetate—15 g.                                 |                     |     |
| Make up with water to—1000 ml.                       |                     |     |
| Then add glacial acetic acid to pH 4.0.              |                     |     |
| 60 Rinsing in water 8 minutes.                       |                     |     |
| Bleaching bath—treatment time 4 minutes:             |                     |     |
| Sodium hexametaphosphate                             | -----               | 5   |
| Potassium ferricyanide                               | -----               | 60  |
| KBr                                                  | -----               | 15  |
| 65 Disodium phosphate                                | -----               | 1   |
| Water up to 1000 ml.                                 |                     |     |
| Rinsing 4 minutes.                                   |                     |     |
| Fixing-bath—treatment time 6 minutes:                |                     |     |
| Sodium thiosulfate cryst.—200 g.                     |                     |     |
| Water up to—1000 ml.                                 |                     |     |
| 70 Rinsing again for 4 minutes.                      |                     |     |
| Final bath in wetting agent—treatment time 1 minute. |                     |     |

A suitable wetting agent bath is, for example, an approximately 0.1% aqueous solution of the sodium salt of paraffin sulfonic acid.

Processing is continued as under A, including the short stop bath.

#### Processing Method D

##### Processing Method B

Color developer as under A—development time 10 minutes.

The same as method A but without the short stop bath. The results of the sensitometric test are shown in the following table:

TABLE

|                                   | A                |                  |                  | B               |         |      | C      |         |      | D       |         |      |
|-----------------------------------|------------------|------------------|------------------|-----------------|---------|------|--------|---------|------|---------|---------|------|
|                                   | Yellow           | Magenta          | Cyan             | Yellow          | Magenta | Cyan | Yellow | Magenta | Cyan | Yellow  | Magenta | Cyan |
| Relative sensitivity <sup>1</sup> | ( <sup>2</sup> ) | ( <sup>2</sup> ) | ( <sup>2</sup> ) | +1              | +1      | +1.5 | +3     | +3      | +4   | +1.5    | +1.5    | +2   |
| Fog                               | 0.23             | 0.18             | 0.16             | 0.28            | 0.20    | 0.18 | 0.32   | 0.22    | 0.22 | 0.32    | 0.29    | 0.26 |
| Gamma                             | 0.69             | 0.62             | 0.66             | 0.67            | 0.60    | 0.64 | 0.62   | 0.57    | 0.60 | 0.62    | 0.60    | 0.60 |
| Grain                             | Standard         |                  |                  | Same to coarser |         |      | Finer  |         |      | Coarser |         |      |

<sup>1</sup> In 0.1 log I.t. units (DIN).

<sup>2</sup> Standard.

After development bath—treatment time 4 minutes: G.

Sodium sulfate ----- 30

KBr ----- 0.25

Make up to 1000 ml., and adjust pH to 10.0.

The procedure is then continued as in Method A, including the short stop bath.

##### Processing Method C

Color developer as under A—development time 10 minutes.

After treatment bath according to the invention—treatment time 4 minutes:

Borax—15 g.

KBr—0.5 g.

Sodium sulfite sicc.—2 g.

Hydroxylamine—2 g.

1-phenylpyrazolidone-(3)—150 mg.

Make up to 1000 ml. and adjust pH to 9.25.

The above figures represent average values obtained from several measurements. The superiority of processing method C according to the invention is readily apparent.

What is claimed is:

1. In the process for producing color-photographic images in complementary colors from a negative film by developing exposed color-photographic material with a color-forming, developer of the p-phenylene diamine series, then bleaching and fixing the developed material, the improvement according to which the color-developed color-photographic negative material has its sensitivity increased and its image grain size reduced by treating it after the color developing bath and before bleaching with an aqueous alkaline bath containing 0.01—1 g. per liter of a black-white developer of the p-aminophenol or 1-phenylpyrazolidone series.

2. The combination of claim 1, wherein the aqueous alkaline bath has a pH of between 8 and 12.

3. The combination of claim 1 in which the aqueous alkaline bath has a pH between 9 and 10.

#### References Cited

#### FOREIGN PATENTS

811,185 4/1959 Great Britain ----- 96—55

NORMAN G. TORCHIN, Primary Examiner

A. T. SURO PICO, Assistant Examiner

U.S. Cl. X.R.

96—55